

Jan. 5, 1926.

1,568,369

S. J. EVERETT

PRODUCTION OF METAL TUBING AND OF TUBULAR METAL ARTICLES OR INSTRUMENTS

Filed Oct. 20, 1923



Fig. 1.



Fig. 2.



Fig. 3.

Inventor  
Samuel James Everett.  
By Henry Orth Jr. act.

Patented Jan. 5, 1926.

1,568,369

# UNITED STATES PATENT OFFICE.

SAMUEL JAMES EVERETT, OF THORNTON HEATH, ENGLAND.

## PRODUCTION OF METAL TUBING AND OF TUBULAR METAL ARTICLES OR INSTRUMENTS.

Application filed October 20, 1923. Serial No. 669,786.

To all whom it may concern:

Be it known that I, SAMUEL JAMES EVERETT, a subject of the King of Great Britain, residing at No. 324 London Road, 5 Thornton Heath, in the county of Surrey, England, have invented certain new and useful Improvements in and Connected With the Production of Metal Tubing and of Tubular Metal Articles or Instruments, of 10 which the following is a specification.

This invention comprises improvements in and connected with the production of metal tubing and of tubular metal articles or instruments. The invention is primarily concerned 15 with the manufacture of tubes of hard or tough metal, such as steel, nichrome and the like, the principal object being to enable tubes of relatively small diameter or gauge to be produced on mandrels or cores 20 which are readily removable from such tubes in spite of the smallness of the bore of the latter. The invention has for a further object to produce in this manner lined tubes of very small diameter, such tubes being 25 advantageous for the manufacture of hypodermic syringe needles.

According to this invention, the tubes are produced by rolling, swaging or drawing a billet containing a mandrel or core of a 30 metal capable of extreme elongation and retention of tensile strength as for example, brass, nickel-silver, and similar alloys. After reduction to the desired gauge or diameter, the severance of a tube length is 35 effected without cutting or breaking the mandrel or core, and the said length is then pulled off from the core the latter stretching and decreasing in diameter and freeing the tube length. In the making of tubes of very 40 small gauge, such as are required for hypodermic syringe needles, a length of tube with its contained mandrel or core is severed, this length being about equal to two needle lengths. The tube length is then divided 45 by severing or breaking one half length from the other without cutting or breaking the mandrel or core and the two half lengths are pulled apart, the stretching and reduction in diameter of the mandrel due to such 50 pulling enabling the separation of the half lengths, or needle lengths, from the mandrel or core to be readily effected. Lined tubes may be produced by interposing a tube of lining metal, such as silver, or nickel-silver, between the billet and mandrel.

This manufacture of tubing is very advantageously adopted in the manufacture of hypodermic needles particularly when these are to be made of the so-called rustless or stainless chrome or like steel. Owing to the 60 smallness of the gauge, it is not practical to impart to the cylindrical wall of the bore the high polish which is imparted to the exterior of the tube or needle and which is necessary for maintenance of the rustless or 65 stainless character of the metal. For this reason, a lining of silver or nickel silver, or like non-corrodible metal is provided in the manner described.

In order to enable the invention to be 70 readily understood, reference will be made to the accompanying drawing, in the course of a description of one suitable method of carrying out the invention. In the drawing:—

Figure 1 is a longitudinal section of a core immediately surrounded by a tube of lining metal which, in turn, is surrounded by a tubular billet of steel or the like.

Figure 2 is an enlarged longitudinal section of a finished tube with its core shown 80 in elevation, the breaking of a length of this tube prior to removal from the core being indicated by broken lines.

Figure 3 is an enlarged perspective view 85 of a hypodermic syringe needle made from a length of tubing such as is seen in Figure 2.

Assuming that stainless steel hypodermic needles are to be manufactured, a mandrel or core *a* of brass or nickel silver, of suitable length and diameter, is coated with graphite *b* or the like, and a length *c* of silver, nickel silver, or other incorrodible lining metal is passed on to the mandrel or core *a*. The exterior of the tube length *c* 90 is coated at *d* with borax or like flux and it may also be coated with a solder. The mandrel or core *a* with its enclosing tube of lining metal *b* is now inserted into the bore of the tubular billet *e* of stainless or chrome steel and this composite object is subjected to rolling, swaging or drawing for the production of a tube of the desired gauge, as for example the tubular needle *f* for a hypodermic syringe, such as is seen in Figure 105 3.

The tube is subjected to heat treatment for annealing the mandrel *a* and the combined effect of the rolling, swaging, or drawing and heat treatment causes the lining *c* 110

to be welded, soldered or intimately allied with the interior of the steel tube, whereby such interior is protected and will not corrode, although not of a polished nature. In 5 Figure 2, the lining of the tube after the rolling, swaging or drawing and heating is seen to be merged into the outer steel and is indicated by dotted lines.

A length of tubing with its contained core 10 equal to about two needle lengths is now cut off. This length of tube is severed in the middle, or is broken at that point by judicious bending as illustrated at *g* in Figure 2, but without cutting or breaking the core 15 *a*, and the two half-lengths, or two needle lengths, (one needle length being indicated in chain lines at *h* in Figure 2) are pulled apart. The elongation and reduction in diameter of the core *a* due to the pulling, 20 enables a clean separation of the interior of the needle lengths from the core to be effected.

Alternatively, the main length, such as 25 the length to the left hand side of the break *g* in Figure 2, may be suitably held and a desired length, such as the needle length *h* of the tube only is severed or broken and pulled off, as will now be readily understood.

30 I claim:—

1. The production of a lined steel tube of 35 small gauge consisting in the reduction to small gauge of a composite billet comprising an outer steel tube, an inner tube of non-corrodible metal, a core of metal capable of extreme elongation and retention of tensile strength, and a uniting medium between said outer and inner tubes, subjecting said tubes and core to a heat treatment, severing 40 a length of the finished tube but not the core and removing said length of tube from the core by a pulling operation which extends said core, substantially as set forth.

2. The production of hard metal tube 45 lengths consisting in the reduction to small gauge of a tubular billet containing a core of metal capable of extreme elongation and retention of tensile strength, severing a length of the finished tube but not the core,

and removing said length by a pulling operation which extends said core substantially as set forth. 50

3. The production of tubular steel instruments consisting in the reduction to small gauge of a composite billet composed of an outer steel tube, an inner tube of non-corrodible metal and a core of metal capable of extreme elongation and retention of tensile strength, subjecting the said tubes and core to a heat treatment, severing a length 55 of the finished tube but not the core, and removing said length by a pulling operation which extends said core substantially as set forth. 60

4. The production of a hypodermic 65 syringe needle from a composite billet comprising an outer tube of stainless steel, an inner lining tube of non-corrodible non-ferrous metal, and a core of metal capable of extreme elongation and retention of tensile 70 strength, consisting in the reduction to small gauge of said composite billet, subjecting said tubes and core to heat treatment for uniting said outer tube and said lining tube, severing a needle length of said tube without 75 severing said core, and removing said length by a pulling operation which extends said core substantially as set forth. 75

5. The production of hypodermic syringe 80 needles from a composite billet comprising an outer tube of stainless steel, an inner lining tube of non-corrodible non-ferrous metal and a core of metal capable of extreme elongation and retention of tensile 85 strength, consisting in the reduction to small gauge of said composite billet, subjecting said tubes and core to heat treatment for uniting said outer tube and said lining tube, severing from the small gauge tubing and 90 core a portion equal to two needle lengths, effecting a breakage in the tubing of said portion between its ends without breaking the contained core, and effecting removal of the tube portions from the core by pulling them apart and extending said core substantially as set forth. 95

SAMUEL JAMES EVERETT.